

Jan. 15, 1929.

1,699,349

W. B. DAILEY

METHOD OF AND MEANS FOR MAKING PHOTOGRAPHIC PAPER, FILM OR THE LIKE

Filed Feb. 1, 1924



INVENTOR:

William B. Dailey,  
BY  
Everett Park,  
ATTORNEYS.

Patented Jan. 15, 1929.

1,699,349

# UNITED STATES PATENT OFFICE.

WILLIAM B. DAILEY, OF EAST ORANGE, NEW JERSEY.

METHOD OF AND MEANS FOR MAKING PHOTOGRAPHIC PAPER, FILM, OR THE LIKE.

Application filed February 1, 1924. Serial No. 689,929.

The objects of this invention are to apply a light-sensitive coating and a protective coating to a photographic medium base, such as paper, film or other sheet material, in one and the same operation; to enable the two coatings to be dried at the same time, and thus equally in finishing the product; to save time, labor, expense, apparatus and space therefor, and to obtain other advantages and results as may be brought out by the following description.

Referring to the accompanying drawing, the single figure thereof is a diagrammatic illustration of one means for carrying out my improved method.

It will be understood that my improvements can be utilized in connection with any light-sensitive photographic medium, comprising a base such as paper, film, or any other kind of a sheet, to which a light-sensitive coating of any kind is applied, such as gelatine with which any light-sensitive salt, such as silver, platinum or other usual substance, has been incorporated, and upon which coating it is desired to superpose a second coating which shall protect the light-sensitive coating against abrasion, friction marks and the like caused by contact of objects with said light-sensitive coating, for example, a second coating of non-sensitized gelatine.

To illustrate my invention, I have shown in the drawing a roll 1 of paper or any other suitably flexible sheet material to be coated upon its side 2, and have shown such sheet material led through suitable feeding and tension rolls 3 to a coating roll 4, where the sheet material dips its surface 2 into sensitized gelatine 5, of any well-known kind, in a container 6 which can be adjusted toward and away from the roll 4, as by slots 7, and is warmed in any ordinary and well-known manner to keep the gelatine liquid. From this coating roll 4 the sheet material is directed as by rollers 8 and 9 to a cooling chamber or duct 10 which serves to set the gelatine coating sufficiently to receive the second or unsensitized protective coating. For this purpose, the sheet material after leaving the cooling chamber 10 passes to a second coating means which applies to the already coated side of the sheet material a second coating, preferably gelatine, which is unsensitized and adapted to be applied similar to the first coating. For convenience I have shown this coating applied by a roll

11 from a container 12 which is adjustable by means of slots 13, similar to the first coat-applying means, but it might be of any other construction commonly used for applying coatings. After receiving this second coating the sheet material passes through a cooling chamber or duct 14 to set the coating, and then after leaving a directing roller 15 it is looped and thoroughly dried in the usual manner for packaging, as at 16.

The setting of each coating immediately after it has been applied does not dry it, but is merely a chilling; the two coatings are dried at the same time, as at 16 in the drawing, and are thus dried equally so that the photographic medium is uniform throughout in that respect.

It will be noted that the means for applying the successive coatings to the sheet material are at the same side of the path of the material and that the means for supporting the material while so coated are all at the opposite side of the path of the material, so that the first coating does not engage anything solid before the second coating is applied and therefore cannot be marred in any way. If the coatings were dried separately, so that the material with its first coat were rolled, said coating would be damaged so as to greatly impair the photographic material, and by my improved method of drying both coatings at once I enable such rolling to be avoided.

Any suitable means may be employed for causing the sheet material to unwind from the roll 1 and travel over its coating rolls, through the cooling chambers and so forth until it is ready for packaging, and I have indicated such means by a belt 17 from a driving member 18 extending to a pulley 19 on the same shaft with the roller 8 and a belt 20 extending from another pulley 21 on said shaft to a pulley 22 on the same shaft with the roller 15.

While I have shown for illustrative purposes one means for producing my improved photographic paper, film or the like, I desire to point out that the coatings can be applied in any other suitable and well-known manner than by the rolls shown, and either the same or different means can be used for the two coatings. Furthermore, various kinds of sheet material and of coatings, either sensitive or protective, may be employed by those skilled in the art, without departing from the spirit and scope of the invention,

and I do not wish to be understood as limiting myself except as required by the following claims when construed in the light of the prior art.

5 Having thus described the invention, what I claim is:

1. The method of making a light-sensitive photographic medium, which consists in applying to sheet material a light-sensitive coating, causing the same to set, superposing a protective coating upon said sensitive coating while so set and before it is dry, and drying both said coatings at the same time.

10 2. The method of making a light-sensitive photographic medium, which consists in applying to sheet material a light-sensitive coating, causing the same to set, superposing upon said sensitive coating while so set and before it is dry a protective coating of the same body material, and drying both said coatings at the same time.

15 3. The method of making a light-sensitive photographic medium, which consists in applying to sheet material a light-sensitive gelatine coating, causing the same to set, superposing a protective gelatine coating upon said sensitive gelatine coating while so set and before it is dry, and drying both said coatings at the same time.

20 4. The method of making a light-sensitive photographic medium, which consists in applying to sheet material a light-sensitive coating in warm liquid condition, chilling the same to cause it to set, superposing a protective coating upon said sensitive coating while so set and before it is dry, and drying both said coatings at the same time.

25 5. The method of making a light-sensitive photographic medium, which consists in applying to sheet material a light-sensitive coating in warm liquid condition, chilling the same to cause it to set, superposing upon the sensitive coating while so set and before it is dry a protective coating in warm liquid condition, chilling said second coating to cause it to set, and drying both said coatings at the same time.

30 6. The method of making a light-sensitive photographic medium, which consists in applying a light-sensitive coating to sheet material, applying a protective coating to said light-sensitive coating before it is dry, and drying said coatings at the same time.

35 7. The method of making a light-sensitive photographic medium, which consists in applying a light-sensitive coating to sheet material, applying a protective coating to said light-sensitive coating before it is dry, and drying said coatings.

40 8. The method of making a light-sensitive photographic medium, which consists in applying to sheet material a light sensitive coating, causing said coating to set, applying a protective coating to said light-sensi-

tive coating before it is dry, causing said protective coating to set and drying both coatings at the same time.

9. The combination with means for applying a light-sensitive coating to sheet material, means for drying the coated material, and means for conveying said material from said coating means to said drying means, of means for applying a protective coating upon said light-sensitive coating before the sheet material reaches the drying means and far enough beyond the means for applying the light-sensitive coating for said coating to have set.

10. The combination with means for applying a light-sensitive coating to sheet material, means for drying the coated material, and means for conveying said material from said coating means to said drying means, of means for applying a protective coating upon said light-sensitive coating before the sheet material reaches the drying means, and means between said means for applying the light-sensitive coating and means for applying the protective coating for causing the light-sensitive coating to set.

11. The combination with means for applying a light-sensitive coating to sheet material, means for drying the coated material, and means for conveying said material from said coating means to said drying means, of means for applying a protective coating upon said light-sensitive coating before the sheet material reaches the drying means, means between said means for applying the light-sensitive coating and means for applying the protective coating for causing the light-sensitive coating to set, and means between said means for applying the protective coating and means for drying for causing said protective coating to set.

12. The process of forming a photographic film which comprises applying to a sheet a liquid coating of sensitized emulsion, only partially hardening said coating, applying to said coating a protective liquid coating, and drying the film so formed.

13. The process of forming a photographic film which comprises applying to a sheet a liquid coating of sensitized emulsion, chilling said coating without drying it, applying to said coating while wet a protective liquid coating and drying the film so formed.

14. The process of forming a photographic film which comprises coating a sheet with sensitized emulsion, partially hardening said coating, and applying thereto before drying a protective liquid coating, hardening said liquid coating, and then drying the film so formed.

15. An apparatus for forming photographic films, comprising means for coating a sheet with sensitized emulsion, a cooling device adapted to receive said sheet from said means, means for coating said emulsion

before drying and adapted to directly receive the sheet from said cooling means and apply the second coating while the emulsion is still wet, a second cooling means 5 adapted to receive the sheet from said last named means, and film drying means for receiving the sheet from said second cooling means.

16. An apparatus for forming photographic films, comprising means for coating a sheet with sensitized emulsion, a cooling device adapted to receive said sheet from said means, means for coating said emulsion before drying adapted to directly receive the 10 sheet from said cooling means and apply the second coating while the emulsion is still wet, a second cooling means adapted to receive the sheet from said last named means, and film drying means for receiving the sheet from said second cooling means, said 15 apparatus being constructed to maintain the coated surfaces of said sheet free from contact with any portion of said apparatus.

17. In an apparatus for forming a photographic film, a container providing a bath 25 for coating one side of the film with an emulsion, intermediate coating means partially hardening the coating without drying it, a container providing a second bath for applying a second coating to the same side 30 of said film while the emulsion is still wet, and guiding means for receiving the said film from the first bath container and delivering the same to the second bath container, said guiding means engaging only 35 the uncoated side of said film throughout all of said operations.

18. The process of forming a photographic film comprising applying a fresh emulsion film to the film base, setting said film by 40 refrigeration and then immediately applying an outer protective coating, cooling both coatings together to set them, and drying the compositely coated film.

WILLIAM B. DAILEY.